

June 24, 1930.

J. MAHLER

1,768,125

PROCESS OF PRODUCING PATTERNS ON PLATED KNITTING  
AND THE CORRESPONDING PRODUCT

Filed Oct. 10, 1927

Fig. 1.



Fig. 2.



Inventor:  
Josef Mahler  
By his Attorney:  
Hauson & Guron

## UNITED STATES PATENT OFFICE

JOSEF MAHLER, OF NEMECKY BROD, CZECHOSLOVAKIA, ASSIGNOR TO FIDELITY MACHINE COMPANY, OF PHILADELPHIA, PENNSYLVANIA, A CORPORATION OF DELAWARE

## PROCESS OF PRODUCING PATTERNS ON PLATED KNITTING AND THE CORRESPONDING PRODUCT

Application filed October 10, 1927, Serial No. 225,402, and in Czechoslovakia July 1, 1927.

It is known in connection with woven fabrics to produce patterns by a process of carbonization wherein part of the texture is destroyed by means of corrosive agents.

The present invention consists in applying the above process to plated stockings or other plated knitting, the two web portions being made of different kinds of materials such as cotton and wool so that a patterning can subsequently be produced by applying to the top surface, for instance by printing, a corrosive which only attacks the plating and leaves the ground work to appear through the latter.

In this manner a Jacquard effect can be produced by very simple and inexpensive means.

By the present process, it is possible to obtain a design outlined by a sharply defined line which will follow a predetermined configuration irrespective of the outline of the individual stitches of the foundation fabric. Designs have been knit into the fabric by means of plating, but it has never been possible heretofore to produce a design in a knitted fabric in which the outline of the design will follow a sharply defined line, for, of necessity, the knitted design is defined by the outlines of the individual stitches of the foundation fabric upon which the plating stitches are laid, the plating stitches assuming the same form as that of the underlying foundation stitches. With the present invention, however, if desired, the outline of the design may be made to cut across the plating stitches, a portion of the stitch being removed while the remaining portion constitutes a part of the sharply defined line.

For the etching out of the cotton, the pattern is printed with sulphuric acid. A solution of caustic soda may be used for etching out the wool.

In the accompanying drawing, Figures 1 and 2 respectively illustrate pieces of plated knit goods 1, having areas 2 of predetermined outline in which the plating has been removed, in accordance with the process above set forth, leaving the groundwork 3 exposed to view. In Figure 2, the outlines 4 and 5 of the areas 2 are shown as cutting across the plated stitches 6, thereby sharply defining

the outlines of the plated areas 7 irrespective of the outlines of the individual stitches of which the fabric is composed.

## I claim:

1. A process of producing patterns on plated knitting consisting in forming the plating and the ground work out of different materials, and printing the pattern on the knitting with a corrosive agent adapted to destroy the plating material without attacking the ground work. 55

2. A process of producing patterns on plated knitting consisting in forming the ground work out of wool and the plating out of cotton, and printing the pattern on the knitting with sulphuric acid. 65

3. The process of producing designs on plated knitting, outlined by a sharply defined line following a predetermined configuration irrespective of the outlines of the individual stitches of the foundation fabric, the ground work of the plated knitting being of one material and the plating of another material which comprises exposing a portion of the plated knitting to the action of a corrosive agent adapted to destroy the plating in predetermined areas according to the design desired without attacking the ground work or the plating of other areas, allowing the corrosive agent to act upon and destroy the susceptible plating material in the predetermined areas to which it is applied, and thereafter freeing the fabric of the corrosive agent. 70 75 80

4. A process of producing patterns on plated knitting, the groundwork being of one material and the plating of another material, which comprises exposing a portion of the plating to the action of a corrosive agent adapted to destroy the plating in predetermined areas according to the design desired without attacking the groundwork, allowing the corrosive agent to act upon and destroy the susceptible plating material in the predetermined areas to which it is applied, and thereafter freeing the fabric of the corrosive agent. 85 90 95

5. A plated knitted fabric, the plating of which is of one material while the groundwork is of another material having a design 100

formed thereon, the plating having been removed in predetermined areas by a corrosive agent which destroyed the plating without attacking the groundwork, the groundwork appearing through the plating in the said predetermined areas to form the design.

6. A plated knitted fabric, the plating of which is of one material while the groundwork is of another material having a design thereon outlined by a sharply defined line following a predetermined configuration irrespective of the outlines of the individual stitches of the foundation fabric, the plating having been removed in predetermined areas by a corrosive agent which destroyed the plating without attacking the groundwork, the groundwork appearing through the plating in the said predetermined areas to form the design.
- 10 7. A plated knitted fabric, the plating of which is of one material while the groundwork is of another material having a design formed thereon, the plating having been removed in predetermined areas by a corrosive agent which destroyed the plating without attacking the groundwork to form a predetermined design.
- 15
- 20
- 25

JOSEF MAHLER.

30

35

40

45

50

55

60

65